

# UNITED STATES PATENT OFFICE.

FRANK CAMERON, JR., OF HARRISON, OHIO, ASSIGNOR OF ONE-THIRD TO FRANK SINGER, OF HARRISON, OHIO.

## STOVE-POLISH.

1,094,302.

Specification of Letters Patent.

Patented Apr. 21, 1914.

No Drawing.

Application filed January 7, 1913. Serial No. 740,675.

*To all whom it may concern:*

Be it known that I, FRANK CAMERON, Jr., citizen of the United States, residing at Harrison, in the county of Hamilton and 5 State of Ohio, have invented certain new and useful Improvements in Stove-Polish, of which the following is a specification.

My invention relates to new and useful improvements in polishing compounds and 10 the object of my invention is to provide a non-inflammable stove polish of superior quality.

A further object of my invention is to provide a stove polish which may be used 15 with equal effect as a cleaning polish for cleaning nickel-plated ware, silver ware and blue steel. This polish may also be used to polish rusty iron and cast iron and when so used will give the articles a dull black finish, 20 the polish being therefore particularly adapted for use with iron andirons.

My stove polish is preferably formed from the following ingredients in substantially the 25 proportions set forth, although these proportions may be varied slightly without departing from the spirit of my invention.

|                            |          |
|----------------------------|----------|
| Ives Family Soap (38 bars) | 17½ lbs. |
| Graphite                   | 50 lbs.  |
| Gas black                  | 12½ lbs. |
| Water                      | 2 gals.  |
| Turpentine                 | 1 pt.    |
| Oil of sassafras           | ½ pt.    |

35 The Ives Family Soap which, as above indicated, constitutes one of the ingredients of

the compound of this invention, is made up of the following ingredients, in substantially the proportions set forth, although these proportions may, of course, be slightly varied without departing from the spirit of 40 my invention:

|              |              |
|--------------|--------------|
| Moisture     | 5.95 pounds  |
| Silica       | .612 pound   |
| Soda         | .051 pound   |
| Neutral soap | 9.928 pounds |

45

In compounding my improved stove polish, the soap is fully dissolved in the water which is heated to boiling point for that purpose and the other ingredients of 50 the polish are then added. The compound is then thoroughly mixed before it becomes cool. Upon cooling the compound forms a jelly or paste.

The above formula will make between 55 seventy-five and one-hundred pounds of polish. When cool, the polish may be packaged in tin cans or other suitable containers for market.

Having thus described the invention, what 60 is claimed as new is:

A polish including silica, soda and neutral soap, graphite, gas black, water, turpentine, and oil of sassafras.

In testimony whereof I affix my signature 65 in presence of two witnesses.

FRANK CAMERON, JR.

Witnesses:

HORACE G. BOWLES,  
WM. H. MORTASHED.

Copies of this patent may be obtained for five cents each, by addressing the "Commissioner of Patents, Washington, D. C."